

Dec. 5, 1944.

S. D. WELLS

2,364,177

## MANUFACTURE OF BLEACHED KRAFT PULP

Filed May 1, 1942

Fig. 1.



Fig. 2



*Inventor*  
Sidney D. Wells

By: Loans, Pond & Anderson  
Atty's.

## UNITED STATES PATENT OFFICE

2,364,177

## MANUFACTURE OF BLEACHED KRAFT PULP

Sidney D. Wells, Combined Locks, Wis., assignor to The Institute of Paper Chemistry, Appleton, Wis., a corporation of Wisconsin

Application May 1, 1942, Serial No. 441,258

6 Claims. (Cl. 92—9)

The present invention relates to the manufacture of bleached kraft pulp, and more particularly to an improved process of preparing bleached kraft fiber using salt ( $NaCl$ ), lime ( $CaO$ ) and sulfur (S).

In the manufacture of bleached kraft pulp from coniferous woods the wood chips are first cooked in an aqueous bath containing sodium sulfide ( $Na_2S$ ) and sodium hydroxide ( $NaOH$ ), and then after washing are subjected to multi-stage bleaching. The cooking operation carried out in a digester, ordinarily follows the conventional procedure used in the manufacture of unbleached pulps except for more drastic cooking conditions, longer duration of cook, more careful washing, etc. The bleaching operation ordinarily calls for an initial chlorination step followed by a subsequent alkaline hypochlorite step such as described in the bleaching process of Wells Patent No. 1,883,193.

It is universal practice, due to the high cost of chemicals, to recover the sodium base from the black liquor remaining after the cooking treatment. With modern recovery units the make-up chemical required to compensate for the loss in the cooking and recovery cycle is approximately two hundred and fifty (250) pounds of sodium sulfate ( $Na_2SO_4$ ) per ton of kraft pulp. This chemical, which is known in the art as "salt cake," is reduced in the recovery or smelting furnace to sodium sulfide ( $Na_2S$ ) in the presence of black liquor carbonaceous matter.

Heretofore, kraft mills for the most part have purchased chemicals such as salt cake ( $Na_2SO_4$ ), as well as chlorine and caustic soda used in bleaching, on the open market. These materials are relatively expensive and their use (particularly the 1 ton of salt cake needed for 8 tons of pulp) has determined to a large extent the final cost of kraft pulp. Many suggestions have been made with reference to chemical sources but up to the time of the present invention attempts to provide a balanced kraft operating system have been unsuccessful.

The principal object of the present invention is to provide a well balanced operation adaptable for use in the manufacture of bleached kraft pulp.

Other objects will be apparent as the description hereinafter proceeds.

The process of the present invention which includes sodium hydroxide formation by causticizing black liquor smelt, calls for the electrolyzing of common salt, i. e., sodium chloride, re-

sulting in the production of electrolytic hydrogen and chlorine and sodium hydroxide. The chlorine produced in this process is sufficient to provide for both the chlorination and the hypochlorite treatments, and the total sodium hydroxide is sufficient to provide for make-up caustic soda, alkaline extraction, maintain alkalinity during bleaching, etc. The sodium hydroxide is also sufficient when used with sulfur and the by-product hydrogen to provide for make-up sodium sulfide. This last step, which is described in detail below makes it unnecessary to use any salt cake in the process of the present invention.

15 The drawings, which are in the form of flow diagrams, will serve to illustrate the present invention. Figure 1 illustrates a complete system, while Figure 2 illustrates a modification of a portion thereof. In Figure 1 the wood chips 10 are first cooked in the conventional manner in digesters 10 in the presence of aqueous sodium hydroxide and sodium sulfide. After cooking the usual washing operation is carried out in washers 11 and the digested unbleached pulp 25 passed on by way of screens and riffles 12 to chlorinator 13.

The black liquor obtained from washers 11 may be treated as shown to recover the sodium base used for digestion. This process includes 30 concentration of the black liquor in concentrator 20, treatment of the concentrate in boiler furnace and smelter 21, treatment of the resulting smelt in dissolver 22 and formation of caustic soda from the green liquor containing the smelt water-solubles in causticizer 23. The sodium compounds in the smelt coming from smelter 21 ordinarily contain small amounts of sodium thiosulfate ( $Na_2S_2O_3$ ) and sodium sulfite ( $Na_2SO_3$ ), somewhat larger amounts of sodium hydroxide and sodium sulfate, about 40 15-20% sodium sulfide and approximately 75% sodium carbonate ( $Na_2CO_3$ ). The sodium hydroxide formed in the causticizer 23 by treatment with quick lime may be illustrated by the 45 following formula:



The insoluble calcium carbonate ( $CaCO_3$ ) sludge formed during this treatment may be removed 50 after settling, and the water solution or fresh white liquor containing the desired proportion of caustic soda passed to digesters 10 for a repetition of the cycle.

The electrolyzing of the salt may be carried 55 out in electrolytic cells 30. Part of the chlorine

obtained by this process is passed to chlorinator 13 for chlorination of the digested pulp, and the remainder of the chlorine is passed to absorber 31 where it reacts with slacked lime ( $\text{Ca}(\text{OH})_2$ ) to produce calcium hypochlorite ( $\text{Ca}(\text{OCl})_2$ ). The chlorinated pulp is washed in washer 14 and subjected to alkaline extraction in alkaline extractor 15—the caustic soda for the last treatment being obtained from the electrolysis of the salt. After alkaline extraction the pulp is washed in washer 16 and is then passed to bleacher 17 for treatment with the calcium hypochlorite formed in absorber 31. During this treatment the desired alkalinity may be maintained in bleacher 17 by use of a portion of the caustic soda formed during electrolysis. The bleached pulp is then subjected to a final washing in washer 18 to obtain the bleached fibers in the desired condition for use in paper making.

The sodium hydroxide obtained from electrolytic cells 30 is passed to concentrator 32 and the resulting concentrate passed on to absorber 33. Portions of the caustic soda concentrate are also passed to alkaline extractor 15 and bleacher 17 as indicated above. The hydrogen from electrolytic cells 30 is passed to retort 34 where it reacts with (gaseous) sulfur heated to a temperature around  $390^\circ \text{C}$ . and forms hydrogen sulfide ( $\text{H}_2\text{S}$ ). The hydrogen sulfide is then passed to absorber 33 which may include scrubbing towers where it reacts with the electrolytic caustic soda to form the desired sodium sulfide. These reactions may be illustrated by the following formulas:



The sodium sulfide solution is then passed to digesters 10 where it is mixed with the caustic soda solution obtained from causticizer 23 and is ready for a repetition of the cycle with fresh wood chips.

An alternative procedure in a portion of the system is illustrated by Figure 2. In this modification the sodium hydroxide or a predetermined portion thereof coming from concentrator 32 is conveyed as fresh white liquor to digesters 10 for use as make-up caustic soda. The sodium hydroxide liquor formed in causticizer 23 is passed to absorber 33' where it reacts as indicated above with the hydrogen sulfide coming from retort 34 to form make-up sodium sulfide. If desired, a portion of the electrolytic sodium hydroxide may be passed as indicated at 35 to absorber 33' in order to enrich the causticized white liquor and provide additional sodium hydroxide for sodium sulfide formation.

The division of the relative amounts of work accomplished between the pulping, purification and bleaching steps is quite flexible. If more alkali is used in the pulping less chlorine is required for chlorination and bleaching. Also the division of what remains to be done after pulping is to a large extent optional. Ordinarily in the preparation of one ton of bleached kraft pulp where the causticized liquor is used for make-up caustic soda, about 200 pounds of chlorine and about 225 pounds of caustic soda are used. With these amounts about 65% of the chlorine is used to chlorinate the unbleached pulp and the remaining (e. g., about 35%) chlorine is used to form calcium hypochlorite; and about 65% of the caustic soda is used to form sodium sulfide and the remaining (e. g., about 35%) caustic soda is used

for alkaline extraction and maintaining alkalinity during the hypochlorite bleach. Of this last amount around three-quarters of the 35% caustic soda (e. g., about 26-27% or 60 pounds) is used in the alkaline extractor and around one-fourth of the 35% caustic soda (e. g., about 8-9% or 20 pounds) is used in the bleacher. A portion of the chlorine may also be used if desired in the water system to prevent slime formation.

It will be understood that the processes outlined in the flow diagrams are merely illustrative and that modifications may be made therein as desired. For example, the active caustic soda in the alkaline extraction liquor may be recovered by passing the liquor to the smelt dissolving tanks, the chlorinated lignin being removed with the calcium carbonate sludge after treatment with lime in the causticizing operation. It will also be understood that an additional hypochlorite bleaching stage may be used and that additional washers may also be used as desired. In the hypochlorite treatments alkalinity (e. g., as shown by the phenolphthalein end point) is maintained by addition of small amounts of caustic soda as the bleach is exhausted. It will also be understood by those skilled in the art that various other modifications may be employed including the recycling of wash waters, the passing of uncombined hydrogen from absorber 33 to retort 34 for combining with sulfur, formation of green liquor in dissolver 22 by use of wash from causticizer 23, etc. In practice the salt ( $\text{NaCl}$ ) impurity in the electrolytic liquor is separated by crystallization in concentrator 32 and returned to the cells as indicated at 36. The various apparatus used in the process of the present invention may be of the standard or conventional type and provide for the addition and removal of water, the use and production of steam, etc.

The process of the present invention which makes the use of relatively expensive salt cake unnecessary may be used in combination with the efficient cooking procedure described in Wells Patent No. 1,949,669. The process of the present invention may also be combined with various other procedures including typical kraft mill digesting, bleaching, recovery, etc., systems to provide a well balanced operation of the type desired. The scope of the present invention should be determined by the claims annexed hereto.

I claim:

1. A balanced system for use in the preparation of bleached kraft pulp which comprises preparing unbleached pulp by cooking wood in a caustic soda-sodium sulfide digesting liquor, preparing a sodium salt smelt by heating the black liquor resulting from the cooking treatment, preparing a green liquor by dissolving the water solubles of the sodium salt smelt, preparing a fresh sodium hydroxide white liquor by a lime causticizing treatment of the green liquor, preparing electrolytic hydrogen and electrolytic chlorine and additional fresh sodium hydroxide white liquor by electrolysis of sodium chloride, preparing a fresh sodium sulfide liquor by reacting the electrolytic hydrogen with sulfur and absorbing the resulting hydrogen sulfide in sodium hydroxide white liquor, and subjecting the unbleached pulp to chlorinating and hypochlorite bleaching treatments, the chlorine for said treatments being electrolytic and being obtained by said electrolysis.
2. In the preparation of bleached kraft pulp the process which includes the following steps (1) cooking wood chips in an aqueous sodium hy-

dioxide-sodium sulfide bath to form unbleached pulp, (2) smelting the black liquor resulting from step (1) to form a sodium salt smelt, (3) electrolyzing aqueous sodium chloride to form chlorine, sodium hydroxide and hydrogen, (4) chlorinating the unbleached pulp of step (1) with part of the chlorine obtained in step (3), (5) subjecting the chlorinated pulp of step (4) to alkaline extraction with part of the sodium hydroxide obtained in step (3), (6) forming calcium hypochlorite by reacting calcium hydroxide with chlorine obtained in step (3), (7) bleaching the alkalized pulp of step (5) by treatment with the calcium hypochlorite obtained in step (6), (8) forming hydrogen sulfide by reacting sulfur with the hydrogen obtained in step (3), (9) forming a sodium sulfide liquor by absorbing the hydrogen sulfide of step (8) in sodium hydroxide obtained in step (3), (10) forming a sodium hydroxide liquor by causticizing the smelt of step (2) by treatment with calcium hydroxide, and (11) mixing the sodium sulfide and sodium hydroxide liquors of steps (9) and (10) respectively for a repetition of the cycle with fresh wood chips.

3. In the preparation of bleached kraft pulp the process which includes the following steps (1) cooking wood chips in an aqueous sodium hydroxide-sodium sulfide bath to form unbleached pulp, (2) smelting the black liquor resulting from step (1) to form a sodium salt smelt, (3) electrolyzing aqueous sodium chloride to form chlorine, sodium hydroxide and hydrogen, (4) chlorinating the unbleached pulp of step (1) with part of the chlorine obtained in step (3), (5) subjecting the chlorinated pulp of step (4) to alkaline extraction with part of the sodium hydroxide obtained in step (3), (6) forming calcium hypochlorite by reacting calcium hydroxide with chlorine obtained in step (3), (7) bleaching the alkalized pulp of step (5) by treatment with the calcium hypochlorite obtained in step (6), (8) forming a white liquor containing sodium hydroxide by causticizing the smelt of step (2) by treatment with calcium hydroxide, (9) forming hydrogen sulfide by reacting sulfur with the hydrogen obtained in step (3), (10) forming additional sodium sulfide by absorbing the hydrogen sulfide of step (9) in the white liquor obtained in step (8), and (11) mixing electrolytic sodium hydroxide obtained in step (3) with the sodium sulfide liquor obtained in step (10) for a repetition of the cycle with fresh wood chips.

4. In the preparation of bleached kraft pulp the process which includes the following steps (1) cooking coniferous wood chips in an aqueous sodium hydroxide-sodium sulfide bath to form unbleached pulp, (2) washing the digested pulp of step (1), (3) concentrating and smelting black liquor resulting from steps (1) and 2) to form a sodium salt smelt, (4) electrolyzing aqueous sodium chloride to form chlorine, sodium hydroxide and hydrogen, (5) chlorinating the washed pulp of step (2) with part of the chlorine obtained in step (4), (6) washing the chlorinated pulp of step (5), (7) subjecting the washed pulp of step (6) to alkaline extraction with part of the sodium hydroxide obtained in step (4), (8) washing the pulp of step (7), (9) forming calcium hypochlorite by reacting calcium hydroxide with chlorine obtained in step (4), (10) bleaching the

washed pulp of step (8) by treatment with the calcium hypochlorite obtained in step (9), (11) maintaining an alkaline condition during the bleaching treatment by addition of part of the sodium hydroxide obtained in step (4), (12) washing the bleached pulp of step (10), (13) forming hydrogen sulfide by reacting sulfur with the hydrogen obtained in step (4), (14) forming a sodium sulfide liquor by absorbing the hydrogen sulfide of step (13) in sodium hydroxide obtained in step (4), (15) forming a sodium hydroxide liquor by causticizing the smelt of step (3) by treatment with calcium hydroxide, and (16) forming a fresh cooking liquor by mixing the sodium sulfide and sodium hydroxide liquors of steps (14) and (15) respectively.

5. In the preparation of bleached kraft pulp the process which comprises forming unbleached pulp by cooking chips of coniferous wood in an aqueous sodium hydroxide-sodium sulfide liquor, washing the unbleached pulp, forming a sodium salt smelt by concentrating and smelting the black liquor produced during the cooking of the chips, forming a green liquor by dissolving in a causticizing wash the water soluble salts contained in the smelt produced by the smelting operation, forming white liquor containing a substantial portion of sodium hydroxide by causticizing the green liquor with quick lime, a wash from this treatment serving as the dissolving medium in the preparation of the green liquor, forming electrolytic chlorine and hydrogen and sodium hydroxide by electrolysis of aqueous sodium chloride, chlorinating the washed unbleached pulp with electrolytic chlorine, washing the chlorinated pulp, subjecting the washed chlorinated pulp to alkaline extraction with electrolytic sodium hydroxide, washing the alkaline extracted pulp, forming calcium hypochlorite by reacting electrolytic chlorine with calcium hydroxide, bleaching the washed alkaline extracted pulp by treatment with the calcium hypochlorite, maintaining the calcium hypochlorite liquor in an alkaline condition during the bleaching treatment by addition of electrolytic sodium hydroxide, washing the bleached pulp, forming hydrogen sulfide by reacting the electrolytic hydrogen with sulfur, forming additional sodium sulfide by absorbing the hydrogen sulfide in the sodium hydroxide white liquor, and forming a fresh cooking liquor by mixing electrolytic sodium hydroxide with the sodium sulfide liquor.

6. In a balanced system adaptable for use in the preparation of bleached kraft pulp, the process which comprises preparing unbleached pulp by cooking wood in a caustic soda-sodium sulfide digesting liquor, preparing sodium hydroxide by causticizing a sodium salt smelt obtained by heating the black liquor resulting from the cooking treatment, preparing chlorine and hydrogen and additional sodium hydroxide by electrolysis of sodium chloride, and preparing a fresh sodium sulfide liquor by the reaction of the hydrogen with sulfur and the reaction of the resulting hydrogen sulfide with sodium hydroxide, said process providing sufficient chlorine for chlorination and bleaching of the pulp and sufficient caustic soda and sodium sulfide for making up fresh cooking liquors.

SIDNEY D. WELLS.